

## UNITED STATES PATENT OFFICE.

CHARLES B. JACOBS, OF WILMINGTON, DELAWARE, ASSIGNEE TO E. I. DU PONT DE NEMOURS & COMPANY, OF WILMINGTON, DELAWARE, A CORPORATION OF DELAWARE.

## ACID-RESISTANT ALLOY.

No Drawing.

Application filed May 6, 1922. Serial No. 559,068.

*To all whom it may concern:*

Be it known that I, CHARLES B. JACOBS, a citizen of the United States, and a resident of Wilmington, in the county of New Castle and State of Delaware, have invented a certain new and useful Acid-Resistant Alloy, of which the following is a specification.

This invention relates to an alloy composed mainly of copper and silicon, and containing a sufficient amount of a third element, as for example manganese, to render the alloy machinable and workable.

The chief object of my invention is to provide an alloy that is extremely resistant to the chemical action of mineral and organic acids and other corrosive liquids, and that at the same time possesses those physical properties, such as high tensile strength and ductility, which will permit of its practical use in the manufacture of reaction-vessels and various other articles or parts of chemical apparatus which are destined to be subjected to the action of corrosive chemical reagents.

I have discovered that by combining copper with silicon, an alloy is obtained having an exceptionally high resistance to the action of liquids which are ordinarily regarded as corrosive. I found that silicon would combine with copper in varying proportions and that there appeared to be definite compounds corresponding to the formula  $Cu_1Si_4$  and  $Cu_8Si$  with a eutectic containing 18% silicon melting at  $810^\circ C$ . Silicon-copper alloys of the above composition, although very acid-resistant, were found, however, to be extremely brittle. Even 5% of silicon combined with copper was found too brittle and weak in structure to meet the uses to which it was intended to put the alloy. I then discovered that the addition of small amounts of manganese toughened and strengthened these alloys so that the products possessed the requisite strength and other physical properties for my purpose without injury to their corrosion-resistant properties.

The alloys made in accordance with my invention may be described as having a base of copper to which appreciable amounts of manganese and silicon have been added for the specific purposes above noted, the silicon predominating over the manganese. The

alloy contains no other elements except incidental impurities, principally iron introduced with the manganese or silicon. Using the technically pure manganese and silicon products now obtainable on the market the highest iron content I have yet found in the new alloy is less than 0.2%. Of the new alloys, those containing from 3 to 6.5% silicon with from .5 to .7% manganese, the balance being copper except for incidental impurities such as traces of iron in the silicon and manganese, were found to be characterized by the physical properties of first-class bronzes and when properly cast showed a tensile strength varying from 34,000 to 42,000 lbs. per square inch with from 10 to 37% elongation and from 18 to 45% reduction of area depending on the manner in which they were cast and somewhat on the relative proportions of silicon and manganese in the alloy. Alloys within these limits are sufficiently ductile to permit their being worked under the proper conditions into sheets, wire and tubing or they may be used in the form of castings made either in green sand or in permanent molds.

Alloys containing from 7 to 15% of silicon with from .8 to 3% manganese are characterized physically by greater hardness and a tensile strength upwards of 48,000 to 50,000 lbs. per square inch with 7 to 12% elongation and from 6 to 12% reduction in area but have hardly sufficient ductility to work well into thin sheets or wire. It, however, would not be proper to state that alloys containing the above higher percentages of silicon can not eventually be worked as well as those containing the lower percentages.

These alloys may be produced by melting a given weight of copper and adding to it pure manganese and pure refined silicon in the desired proportions. It is advisable as in the melting of all bronzes and similar copper alloys to first melt the copper in plumbago crucibles under charcoal to protect it against oxidation and contamination from furnace gases. The best pouring temperature from producing sound castings is in the neighborhood of  $1900-2000^\circ F$ .

The preferred method and the one which gives uniformly the best results is to first produce in the electric furnace or otherwise, an alloy of manganese and silicon con-

taining say for example 15 to 20% manganese and 80 to 85% silicon with a minimum iron and carbon content and to melt the copper in the usual manner and then add 5 the required proportion of the above alloy to introduce the manganese and silicon. In cases where the relative proportions of manganese and silicon in such an alloy as given above is not properly balanced for a 10 specifically desired alloy the proper balance may be reached by adding either pure silicon or pure manganese as the case may demand to the mixture of metals first melted. A more homogeneous alloy is produced in a 15 shorter time by this method of procedure than when the metals are all added separately.

The above combination of copper, silicon and manganese may be regarded as a type 20 of bronze and be designated as a silicon-manganese bronze, and the best results are usually obtained by handling the melting and pouring of the copper as one would handle ordinary bronze of say 90 to 95% 25 copper and 5 to 10% tin. The addition of the same deoxidizing agents such as phosphor-copper, boron-copper, or any of the well known deoxidizers used in the melting and casting of bronzes may be used in 30 amounts varying from 0.5 to 2% with the same beneficial effects on bronzes composed of silicon, manganese and copper so far as physical characteristics are concerned as on ordinary bronze, and used in such small 35 quantities they have no deleterious effect on the acid-resisting properties of the alloy.

These alloys are characterized chemically 40 by extreme resistance to various mineral and organic acids and other corroding liquids. As an example of the resistance of alloys of the above composition to corrosion may be cited the following.

With the alloy submerged in concentrated 45 hydrochloric acid (35-36% HCl), the penetration per month varies from 0.0012" to 0.0025", the latter figure being obtained when the solution is agitated at the rate of 200 R. P. M. In 3 to 25% sulfuric acid the corrosion varies from practically a passive 50 or inert state to 0.0006" penetration per month, the latter figure when the solution is agitated at the rate of 200 R. P. M. The alloys are extremely resistant to dilute hydrochloric acid in the presence of oxidizing 55 agents—as, for example, a 2 to 3% hydrochloric acid in the presence of sodium chloride,—showing practically no loss or gain in weight after exposure for sixteen days to the above solutions at a temperature of 90° C. 60 under conditions of agitation.

There is also little or no action in the presence of ammonium chloride, zinc chloride, free ammonia vapor and hydrogen chloride at temperatures up to 230° C. as instanced 65 by a loss of but 0.03% in weight when sub-

jected to a solution containing the above substances for a period of sixty hours. Steel and cast iron under the same conditions lost respectively 70 and 22% in weight in sixty hours.

In alum solutions up to 30° Bé. at the boiling point, which by hydrolysis liberates free sulfuric acid, the corrosion expressed in "inches penetration per month" amounted to 0.0006". At higher concentrations of 75 alum solutions as for example 50° Bé. at the boiling point the alloys are inert, i. e., no loss or gain in weight.

In lactic acid, both the dark and edible variety of 22% strength, the alloys are inert 80 in both solutions at the boiling point.

Although specific reference has been made above to copper base alloys containing from 3 to 15% of silicon, and from 0.5 to 3% of manganese, it is to be understood that my invention is not limited to alloys in which the constituents fall within these ranges of proportions. In general there should be a sufficient proportion of silicon to render the 85 alloy more resistant to acids and other corroding agents than are copper, brass, and ordinary bronzes, and a sufficient manganese content to render the alloy machinable and workable. The new alloys may be further defined as copper-silicon-manganese alloys 90 in which the copper predominates, and in which the proportion of silicon is a multiple 95 of the proportion of manganese.

I claim:

1. A copper-base alloy in which the copper is combined with sufficient silicon to form 100 an alloy that is more resistant to acids than is pure copper, said alloy also containing a sufficient amount of manganese to render the alloy machinable and workable.

2. An alloy comprising from about 82 to 96.5% of copper, from about 3 to 15% of 105 silicon, and from about 0.5 to 3.0% of manganese, said alloy being machinable and workable and strongly resistant to acids.

3. An alloy comprising from about 92.5 to 96.5% of copper, from about 3 to 6.5% of silicon, and from about 0.5 to 0.8% of manganese, said alloy being machinable and workable and strongly resistant to acids.

4. An acid-resistant alloy comprising from about 3 to 6.5% of silicon, most of the remainder being copper with sufficient manganese to render the alloy machinable and workable.

5. An alloy comprising from about 3 to 6.5% of silicon, and from about 0.5 to 0.8 manganese, substantially all of the remainder being copper, said alloy having a tensile strength of from 34000 to 42000 125 pounds per square inch, with from 10 to 37% elongation, and from 18 to 45% reduction of area.

In testimony whereof I affix my signature.

CHARLES B. JACOBS.